

March 5, 1929.

H. C. FISHER

1,704,125

METAL PLATING NONMETALLIC SUBSTANCE

Filed April 12, 1924



Fig. 1.



Fig. 2.

INVENTOR:

Harry C. Fisher

BY

Leemell Bellin  
ATTORNEYS.

## UNITED STATES PATENT OFFICE.

HARRY C. FISHER, OF CINCINNATI, OHIO, ASSIGNOR TO THE RICHARDSON COMPANY, OF LOCKLAND, OHIO, A CORPORATION OF OHIO.

## METAL PLATING NONMETALLIC SUBSTANCE.

Application filed April 12, 1924. Serial No. 706,193.

My invention relates to processes of forming on non-metallic surfaces, a coating of metal which is not removable from the non-metallic surface. More specifically it relates to forming metal films on bodies coated with asphalt or some other bitumen and keying these films into the bitumen.

My invention is based on the fact that if a metal in finely divided condition is mixed with water and a volatile liquid which is immiscible with water, such as benzol, under proper conditions, and a thorough emulsion formed, then when this emulsion is poured onto water near boiling temperature so that the benzol will be driven off, the metal which has coated or been held within the body of the minute "bubbles" of benzol will float on the surface of the water, in what is apparently a solid metal film. It is also based on the fact that if such a film is brought into contact with an asphalt surface or other bitumen surface that has been rendered tacky or soft by a solvent, the excess of which has practically been driven off, then this film will coat the bituminous surface and key itself into that surface, each particle in contact with the asphalt becoming partially embedded therein, to an extent tantamount to becoming an integral part with the asphalt. Such a film has the same advantages as a finely divided metal freshly precipitated upon a tacky surfaced solid, and has the additional advantage that it is applicable to metals which are with difficulty produced or held in a pure, reduced and nascent state, and permits use of inexpensive reagents, which can be used on a commercial scale, as in plating asphalt coated shingles, paraffin coated cartons and the like.

It is my object to provide a commercial process wherein a film of metal is formed by the action above noted and is practically freed from the presence of the immiscible liquid that is used, such as benzol, by transference to another water surface, and is there caused to unite with and cover a bitumen coated product. The portions of this film which are out of surface contact with the asphalt, exist in a powdery condition. I then cause these particles to unite with each other and with those partially embedded in

the asphalt, to form a solid plate, by an electroplating treatment.

I accomplish my objects by that certain process to be hereinafter more specifically pointed out and claimed and of which a diagrammatic commercial plant is illustrated.

In the drawing:

Figure 1 is a diagram of the coating unit. 60  
Figure 2 is a diagram of a plant, using my process.

I first proceed to make finely divided metal by some suitable process of replacing the metal in some soluble salt thereof, with another metal, and utilizing the precipitated material. In the instance of copper, this may be done by obtaining copper from the sulphate. An emulsifier or film maker is provided into which is placed the spongy metal and benzol and water, and agitation set up. The proportions of water, benzol and metal are easily determined by experiment, as they depend somewhat on the nature of the firm forming machine. The addition of dilute sulphuric and acetic acids will assist in assuring the desired result, which is to form an emulsion of benzol and water, which emulsion will carry the metal or portions thereof. 80

The emulsion is drawn off and passed into a float case. Here the emulsion proper floats to the surface and is floated onto the surface of a body of heated water. I have shown a float case with sluice 1, extending into a tank 2, which has a suitable heater. As the result of this delivery action and the heat of the water, the benzol is liberated from the emulsion and is drawn off through the hood 3, over a portion of the tank, to a 90 benzol condenser, which regains the benzol for subsequent use. 85

In the tank, I provide a roll 4 as a means for drawing the metal film which is formed by the driving off of the benzol, entirely 95 away from the presence of the benzol, as it forms, to the water surface in the portion 5 of the tank, where it will lie quietly on the water surface, will accumulate into a continuous film, and may by this means, be almost entirely freed of benzol. The importance of removal of the metal from benzol lies in the fact that contact with tacky asphalt while in its benzol phase, or in the 100

presence of benzol, would result in the asphalt coating the metal particles.

The process should be carried on so as to get as much copper or other metal onto the surface of the water as possible. This can be judged by the fact that gravity will overcome the surface tension that supports the metal film when too much metal is produced in the floated film.

10 The element to be coated which I have shown as asphalt coated roofing, which may have a slate surface, is brought through a benzol bath, in which, if the roofing is slate surfaced, there should be 15 considerable asphalt in solution. From this bath, which softens the surface of asphalt-surfaced roofing, or deposits a softened asphalt on the surface of the slate-covered roofing, the sheet may be passed 20 through a drier. If desired, benzol fumes may be used to make the asphalt-surface tacky. It is then passed down over a roll so that its tacky surface comes into contact with the metal film in the tank portion 5. 25 I have shown a roll 6 for the purpose. The sheet is then freed from water and any remaining benzol in another dryer. The roll 6 will preferably cause the web to dip down and then return through the liquid, 30 making it possible to take two films, if desired, and the roll will preferably be below the surface so as not to disturb the film by its movement.

This leaves the product with a non-conductive keyed-in body of finely divided metal and with a conductive surface of loose or dusty nature, which can be readily wiped off. I pass the sheet through an electroplater in which the metal in question is being liberated and is deposited on the conductive surface. The dusty coating may be so formed that a very brief electroplating serves to unite all of the metal together into a solid, keyed-in sheet, integral 45 with the asphalt. The sheet is then washed and dried, and may then pass to a shingle cutter, or other cutting device.

This process may be made continuous and is economical in production of metal coated, 50 non-metallic elements.

The reason for departing from known methods of electroplating non-conductive surfaces by a preliminary treatment with carbon or plumbago to give a conductive base on which to build, is that the film is keyed-in, the electroplating is shortened, and all the coating can be of the metallic character desired.

My process may be applied to any surface 60 but without the integral unity of the metal body and the material to which it is applied. It can also be used to give a metal sheen, or color to products of bituminous nature, without the electroplating step.

65 Having thus described my invention,

what I claim as new and desire to secure by Letters Patent, is:—

1. A process of metal coating a non-metallic product which consists in applying a bituminous surface thereto, rendering 70 said surface tacky by means of a solvent, and bringing the product into contact with film of finely divided metal supported on water surface by surface tension, and subsequently electroplating the surface to unite 75 the metal picked up by the tacky surface from the said film.

2. A process of preparing an article having a metal coating which consists in agitating together a finely divided metal, 80 water and a volatile liquid insoluble in water to form a metal-bearing emulsion and depositing said emulsion on heated water thereby driving off the volatile liquid and thereby forming a film of the metal on 85 the surface of the water making the article adhesive, and then bringing the article into contact with the film.

3. A process of preparing an article having a metal coating which consists in agitating together a finely divided metal, 90 water and a volatile liquid insoluble in water to form a metal-bearing emulsion, and depositing said emulsion on heated water thereby driving off the volatile liquid 95 and thereby forming a film of the metal on the surface of the water, making the article adhesive and then bringing the article into contact with the film.

4. A process for metal coating an article having a bituminous surface which consists in wetting the surface with a solvent thereof, drying the surface sufficiently to leave it tacky, forming a metal film on a surface of water by liberating finely divided metal 100 from a metal-bearing emulsion by heating the emulsion on the water surface, bringing the tacky bituminous surface into contact with the film and subsequently electroplating the metal covered surface to form 105 the deposited powdery metal into a solid sheet.

5. A process of incorporating finely divided metal into the surface of a body which consists in forming a coating of 110 bitumen on the body and rendering the coating tacky on the surface, forming a film of finely divided metal on the surface of water, and dipping said body so as to pick up the film of metal upon the tacky 115 coating thereof.

6. A process of incorporating finely divided metal into the surface of a body which consists in forming a coating of 120 bitumen on the body and rendering the coating tacky on the surface, forming an emulsion bearing a finely divided metal, of water, and a volatile liquid insoluble in water, depositing the emulsion on a fluid support under conditions which evaporate 125 130

the volatile liquid, and dipping said body so as to pick up the film of metal upon the tacky coating thereof.

7. A process of metal coating a non-metallic product which consists in applying a bituminous surface thereto, rendering said surface tacky by means of a solvent, and bringing said tacky surface into con-

tact with a film of finely divided metal supported on water by surface tension, and thereafter electroplating the surface to unite the metal picked up from the film into a solid body keyed into the bituminous surface. <sup>10</sup>

HARRY C. FISHER.